

# UNITED STATES PATENT OFFICE.

LOUIS V. LANDAU, OF LOS ANGELES, CALIFORNIA, ASSIGNOR TO LANDAU'S INSTANTANEOUS DUPLICATOR COMPANY, OF LOS ANGELES, CALIFORNIA, A CORPORATION OF CALIFORNIA.

## COPYING-PAD.

1,348,812.

Specification of Letters Patent.

Patented Aug. 3, 1920.

No Drawing.

Application filed December 4, 1919. Serial No. 342,499.

To all whom it may concern:

Be it known that I, LOUIS V. LANDAU, a citizen of the United States, residing at Los Angeles, in the county of Los Angeles and State of California, have invented new and useful Improvements in Copying-Pads, of which the following is a specification:

My invention relates to a composition for copying pads and has for its object to provide a copying pad which is inexpensive of construction and capable of making copies of printed or written matter made by means of any commercial copying ink, whether printing, writing or hectographic ink of any color.

My invention consists in the new composition hereinafter described and claimed, and which is compounded as follows:

20      3½ kgs. of glycerin,  
6 kgs. of kaolin,  
50 grs. sodium carbonate,  
80 grs. barium sulfate,  
250 grs. dextrin.

The composition is compounded in the following manner: The kaolin is placed in a suitable receptacle and a cavity is formed in the center of the mass of kaolin, for a purpose presently to be described. Into another receptacle the glycerin is placed and 25 gently heated, then the dextrin, sodium carbonate and barium sulfate is added and the temperature raised to about 150° F. It is necessary to avoid bringing the mixture to a boil lest destructive reactions occur. With 30 a suitable stirring device the mixture is agitated until a homogeneous mass is formed. The mixture in the second receptacle, prepared as just described, is now placed into the first receptacle containing the kaolin and into the cavity formed therein, and with 35 a suitable stirring device the kaolin is incorporated in the mixture of glycerin, dextrin, sodium carbonate and barium sulfate until the mass is homogeneous.

40      The mass is now spread upon a table in a thin layer and exposed to the atmosphere for a day or two. The composition is of the consistency and color of putty and has a granular texture.

45      The composition is now ready to be used for the copying pad which may consist of a shallow frame having a flat bottom and side walls of small dimensions. The compo-

sition is placed in the frame and compacted by means of a roller or mallet, and to produce a flat polished surface it is only necessary to rub a moistened sponge over the surface.

55      In making a copy from the sheet printed or written with copying ink, or copying pencils, of various colors, it is merely necessary to place the sheet with the printed face downward on the copying pad and press the same firmly against the pad by means of a roller or mallet and remove the printed sheet, when the copying pad will now have 60 an imprint of the printed or written sheet. A blank piece of paper is now placed on the copying pad and suitable pressure exerted thereon. On removing the sheet of 65 paper a copy of the printed matter will appear on the same. Many copies may be made from the same imprint, or imprints may be made from the first few copies that are taken from the copying pad.

70      To restore the copying pad for the next operation it is merely necessary to use a wet sponge to wipe off the imprint.

75      I find it advisable to add crude rubber to my composition in the proportion of about 80 3% of the whole mass, and thoroughly knead and agitate the mass by any suitable machinery until the rubber is thoroughly disseminated throughout the mass and forms a homogeneous mixture therewith. The 85 composition seems to have solvent properties to soften and dissolve the rubber during the agitation referred to. The object of the rubber is to cause the copying pad to last longer and resist wear.

90      The crude rubber is not absolutely essential and may be omitted.

95      It is understood that various changes may be made without departing from the spirit of my invention as claimed.

I claim:

1. A composition for a copying pad for making copies of printed or written matter, comprising kaolin, glycerin, barium sulfate and dextrin.

100      2. A composition for a copying pad for making copies of printed or written matter, comprising the following ingredients in the proportions stated: kaolin 6 kgs., glycerin 3½ kgs., sodium carbonate 50 grs., barium 105 sulfate 80 grs., and dextrin 250 grs.

3. A composition for a copying pad for making copies of printed or written matter, comprising kaolin, glycerin, barium sulfate, dextrin and rubber.
- 5 4. A composition for a copying pad for making copies of printed or written matter, comprising the following ingredients in the

proportions stated: kaolin 6 kgs., glycerin  $3\frac{1}{2}$  kgs., sodium carbonate 50 grs., barium sulfate 80 grs., dextrin 250 grs., and rubber 10 about 3% of the whole mass.

In testimony whereof I have signed my name to this specification.

LOUIS V. LANDAU.